

Patented Mar. 13, 1928.

1,662,701

# UNITED STATES PATENT OFFICE.

WILLIAM H. ELLERINGTON, OF NAPLES, NEW YORK.

RECLAIMING PROCESS FOR USED CRANK-CASE OIL.

No Drawing.

Application filed January 23, 1926. Serial No. 83,400.

The present invention relates to a new and improved process for purifying lubricating oil which has become contaminated by use with various impurities.

In the use of automobiles, tractors, trucks, and internal combustion engines, oil must necessarily be used for lubricating purposes, particularly about the bearings and cylinders of the engines. Owing to the great heat caused by the combustion of the fuel to propel the motors, much of the oil film about the cylinders finally becomes partially, or entirely destroyed for lubricating purposes, and is eliminated through the valves in the form of carbon and gas, yet much of the carbon of the gas and lubricating oil is carried down by the cylinder and rings, helped by the explosion of the fuel, into the oil reservoir or crank case of the motor, and, through the movements of the mechanism of the machine, becomes thoroughly mixed, not alone with the good clean oil of the crank case, but also becomes incorporated with the sand, grit, and road dust that is inhaled along with the air that enters the motor through the carburetor, and crank case breather. Particles of metal, produced by the rubbing of moving parts, also accumulate with the carbon, dust and original impurities of the oil, and thus soon contaminate the lubricant. The lubricant thus becomes unfit, and highly injurious for the purpose for which it was intended. This is the real reason that manufacturers of cars demand that oil should be renewed every five hundred miles, or less, which is often done, and in consequence, millions of gallons of oil is cast on the ground, or in other ways wasted, that through my methods might be reclaimed, made more pure than at first, and turned back into a long life of usefulness in internal combustion engines, or returned to the crank case of the automobile, truck, or tractor, or used to lubricate bearings wherever machinery may be found, for after the black useless oil is purified, cleaned, and reclaimed by my method it may be redistilled to possess such specific gravity as desired.

In describing my method of obtaining the good oil from a fifty gallon barrel of used and discarded oil, I will state that the same procedure will hold good, in greater or less amounts, bearing in mind the same proportions, more or less, as there is nothing vitally exacting within reasonable amounts. In used oil it will be noticed that there is always a

sufficient amount of carbon remaining in suspension in the oil to be noticeable to the unaided eye. An affinity for the carbon, and other waste, and useless matter is prepared that will add some of its own weight to the light and harmful material in the oil, and drag them with itself down beneath the surface of the oil, which will remain on top of all things both suspended in the oil formerly, and all things that were added for the working of the cure.

I take a fifty gallon barrel containing about forty five gallons of used oil, and elevate it three to four feet, and lay it on its side, (or stand it on end if more convenient) with large bung hole up, and small spigot down. I will have, it will be noted, about space sufficient for adding five gallons of purifying solution, which I prepare in the following way using the following ingredients in about or substantially the proportions given:

|                         |         |
|-------------------------|---------|
| Palm or cotton seed oil | 3 lbs.  |
| Caustic soda—94%        | 8 ozs.  |
| Water                   | 16 ozs. |

Dissolve the soda in the water and keep the solution at 90° F. temperature. Warm the palm or cotton seed oil to 90° F. Pour the soda solution into the warmed palm or cotton seed oil in a thin stream, stirring all the time with a wooden spoon or paddle until the mixture becomes thick and smooth. Now add to this

|                 |   |
|-----------------|---|
| Sodium silicate | 8 |
| Talc powder     | 8 |

Mix thoroughly, and the purifier is now ready for use, by simply adding it to the oil to be treated, and stirring, allowing to settle, and then drawing the purified oil from the top with a siphon. It is advisable to first add to the oil about two or three ounces of aqua ammonia, and thoroughly stir and agitate the oil, and then add sufficient water to the oil, soda, and silicate compound so that it will not become quite as thick as sweet cream when at 40° F. This solution is added to the oil to be reclaimed and after thoroughly stirring five to ten minutes the mixture of oil and purifier is allowed to stand and settle from two days to two weeks according to the temperature which will be best at average summer heat. After the oil has been stirred, a quart fruit jar may be

drawn full from the spigot, as a test, and after the jar has been at rest for a sufficient length of time, it will be noted that all the carbon, grit, dust and iron, (some in the form of an oxide) with the original undesirable properties of the oil, will have settled to the bottom and there will be a well defined line of demarkation or line of distinction between the oil and other elements, and from two thirds to seven eighths of good oil may be expected from the amount of one quart. The longer the jar rests the plainer the line of separation becomes, and it should be held in proper light and looked for above the line of the solution, which will be in the very bottom, incorporated with the dust, iron etc.

When all is ready or sufficient separation shall have been found, take a small rubber tube, (a large one might draw too fast and so encourage a mixture of the carbon and oil) about  $\frac{1}{4}$  to  $\frac{1}{2}$  inches bore, and insert one end in the top of the barrel at the large bung, and syphon the oil off into a receptacle below, and as the oil runs the tube may be pushed gradually further into the barrel, and when carbon shows the least trace in the outlet, the tube should be withdrawn, until the oil shows clean, clear and perfect when looked at upon a clear glass held to the light. If by chance a little carbon is drawn by accident with the oil, it will always go to the bottom, as the alkali and silicate of the solution have taken the place with the water, of the oil that impregnated and permeated the carbon, and the carbon is now heavier than the oil. The oil thus purified may also

be redistilled or heated in some manner from 90° F. to 110° F. or more, if a little heavier oil is desired. It may be heated in a copper 40 boiler on an oil stove, in the open air, and the heating discontinued when a blue or dark vapor is noted arising therefrom.

I find that caustic potash or soda with sodium silicate will clean oil. Powdered 45 vegetable or animal oil soap with some silicate and with talc will also renew the life of oil.

After the oil has been drawn from the barrel through the syphon, the water and 50 chemicals may be drawn off through the spigot. Next will be drawn the carbon with some of the used composition which is very useful for dipping posts and to apply to wood to arrest decay or for preservation. 55 The carbon may be washed with warm water, and water drawn off, washed with gasoline and then used as a base for paint, printer's ink, or even as a writing fluid. The carbon thus produced is pure very finely 60 divided carbon, the little quantity of gasoline used in its extraction being allowed to evaporate.

Having described my invention what I claim and desire to secure by Letters Patent 65 is:

The process of removing carbon, dust, grit, sand, metal particles and like impurities from used lubricating oil which comprises intimately mixing lubricating oil containing 70 such impurities with a mixture including soap, sodium silicate and talc.

In testimony whereof I affix my signature.  
WILLIAM H. ELLERINGTON.